



Analysis of this product gave the following results:

Calculated (percent): P, 4.98; Zn, 5.25; S, 10.31. Found (percent): P, 4.8; Zn, 5.1; S, 10.4.

The infrared spectrographic analysis of the product confirmed the presence of a dithiophosphate group.

#### EXAMPLE 4

##### Evaluation of the anti-oxidant properties

The Staeger oxidation test was carried out on a SAE 30 paraffinic mineral oil with a high viscosity index containing the products of this invention or other additives and the results are shown in the following Table 1.

The test consisted in heating in a thermostatic stove maintained at 110° C. the oil containing the additives under examination. A strip of electrolytic copper was immersed in the oil to act as an oxidation catalyst. At regular intervals the variation in the neutralization number, based on the weight in mg. of KOH./g. oil was recorded.

The test was considered completed when there was an increment of 0.25 in the neutralization number. Oxidation tests were also carried out at 150° C. in the same way as those at 110° C. The concentration of the additives according to the invention was constant in each case. The content of phosphorus was 44.10<sup>-4</sup> g. percent, corresponding to 0.7 millimole of dithiophosphate per kg. of solution. The comparative additives were selected from zinc dithiophosphates obtained from aliphatic alcohols and mixtures thereof with 2,6-di-tert.butyl-paracresol in equimolar concentrations based on the additives of the invention.

TABLE 1

| Additive in SAE 30 mineral oil                                                     | Cone. (m. mole/kg. of solution) | Oxidation (hours at 110° necessary to have an increase of the neutralization number of 0.25) | Oxidation (hours at 150° necessary to have an increase of the neutralization number of 0.25) |
|------------------------------------------------------------------------------------|---------------------------------|----------------------------------------------------------------------------------------------|----------------------------------------------------------------------------------------------|
| None                                                                               |                                 | 310                                                                                          |                                                                                              |
| Zn bisbutyl dithiophosphate                                                        | 0.7                             | 810                                                                                          | 120                                                                                          |
| Bis(4-methyl-2-pentyl)Zn dithiophosphate                                           | 0.7                             | 1,120                                                                                        | 140                                                                                          |
| Bis-ethyl Zn dithiophosphate                                                       | 0.7                             | 820                                                                                          |                                                                                              |
| Bis-butyl Zn dithiophosphate                                                       | 0.7                             | 1,350                                                                                        | 250                                                                                          |
| 2,6-di-tert.butyl paracresol                                                       | 2.8                             |                                                                                              |                                                                                              |
| Bis[(3,5-di-tert.butyl-4-hydroxybenzyl)-propyl]Zn dithiophosphate                  | 0.7                             | 1,610                                                                                        | 370                                                                                          |
| Bis(4-methyl-2-pentyl)Zn dithiophosphate                                           | 0.7                             | 1,260                                                                                        | 210                                                                                          |
| 2,6-di-tert.butyl paracresol                                                       | 1.4                             |                                                                                              |                                                                                              |
| (4-methyl-2-pentyl)-(3,5-di-tert.butyl-4-hydroxy-benzyl)-propyl]Zn dithiophosphate | 0.7                             | 1,420                                                                                        | 230                                                                                          |
| Bis-ethyl Zn dithiophosphate                                                       | 0.7                             | 1,250                                                                                        | 270                                                                                          |
| 2,6-di-tert.butyl paracresol                                                       | 0.7                             |                                                                                              |                                                                                              |
| cetyl [(3,5-di-tert.butyl-4-hydroxybenzyl)-propyl]Zn dithiophosphate               | 0.7                             | 1,320                                                                                        | 300                                                                                          |

As can be seen from the oxidation tests recorded in Table 1, the zinc dithiophosphates of the invention have a high anti-oxidant activity, and the synergism existing between the dialkyl zinc dithiophosphates and sterically hindered phenols, increases when the sterically hindered phenol forms part of the dithiophosphate molecule.

#### EXAMPLE 5

##### Anti-wear tests

In the following Table 2, there are shown the results found in tests in tests on the anti-wear characteristics of an oil containing the products of this invention, compared with the same oil containing known commercial additives.

In Table 2, A is the additive of the Example 1, B the additive of the Example 2, C the additive of the Example 3 and D, E and F are different known commercial additives based on zinc dithiophosphates. The tests were carried out with a "Shell 4 ball Wear Tester," each test lasting 60 seconds at a speed of 1200 r.p.m.

TABLE 2

| Additive | Concen-<br>tration,<br>Percent | Base oil,<br>50° C. | Max. load<br>V.E. in absence of<br>seizure (kg.) | Specific<br>pressure with<br>max. load in<br>absence of<br>seizure,<br>kg./cm. <sup>2</sup> |
|----------|--------------------------------|---------------------|--------------------------------------------------|---------------------------------------------------------------------------------------------|
| None     |                                | 2.95                | 55                                               | 18,330                                                                                      |
| A        | 0.4                            | 2.95                | 100                                              | 25,680                                                                                      |
| B        | 0.4                            | 2.95                | 110                                              | 25,890                                                                                      |
| C        | 0.4                            | 2.95                | 105                                              | 26,370                                                                                      |
| D        | 0.4                            | 2.95                | 110                                              | 25,890                                                                                      |
| E        | 0.4                            | 2.95                | 100                                              | 25,680                                                                                      |
| F        | 0.4                            | 2.95                | 110                                              | 26,450                                                                                      |

From Table 2, it can be seen that the additives of the invention have anti-wear characteristics of a similar nature to known additives.

#### EXAMPLE 6

##### Antirust test

In the following Table 3 there are reported the results found in tests on the anti-rust characteristics of oils containing the same additives as Table 2. The tests were carried out according to the method ASTM/D 665-54.

TABLE 3

| Additive | Concen-<br>tration,<br>percent | Base oil,<br>50° C. | Rust grade |
|----------|--------------------------------|---------------------|------------|
| A        | 0.03                           | 2.95                | Absent.    |
| B        | 0.03                           | 2.95                | Do.        |
| C        | 0.03                           | 2.95                | Do.        |
| D        | 0.03                           | 2.95                | Slight.    |
| E        | 0.03                           | 2.95                | Absent.    |
| F        | 0.03                           | 2.95                | Slight.    |

Thus, as can be seen, the additives of the invention generally have a better anti-rust characteristic than known additives.

What we claim is:

1. A compound represented by the following formula:



wherein M is a calcium, barium, nickel, cadmium, or zinc atom; and R, R', R'' and R''' are alkyl radicals containing up to 10 carbons, at least one of R, R', R'' and R''' having the formula:



wherein A is a bivalent hydrocarbon radical containing from 1 to 20 carbon atoms and said hydroxy group is sterically hindered by a vicinal alkyl group containing up to 10 carbons.

2. A compound as claimed in claim 1 wherein said hydroxy group is sterically hindered by vicinally positioned secondary or tertiary alkyl groups.

3. A compound as claimed in claim 1 wherein said hydroxy group is in the para position sterically hindered by vicinally positioned tertiary butyl groups. 5

4. A compound as claimed in claim 1 having the name bis[(3,5 - di-tert.butyl-4-hydroxy-benzyl)propyl] zinc dithiophosphate.

5. A compound as claimed in claim 1 having the name (4 - methyl -2- pentyl)[(3,5-di-tert.butyl-4-hydroxy-benzyl)-propyl] zinc dithiophosphate.

6. A compound as claimed in claim 1 having the name cetyl[(3,5 - di - tert.butyl-4-hydroxy-benzyl)-propyl] zinc 10 15 dithiophosphate.

## References Cited

## UNITED STATES PATENTS

|           |         |                         |             |
|-----------|---------|-------------------------|-------------|
| 2,252,984 | 8/1941  | Rutherford et al. ----- | 252—35      |
| 2,342,572 | 2/1944  | Cook et al. -----       | 260—448 X   |
| 2,480,673 | 8/1949  | Reiff et al. -----      | 252—32.7    |
| 2,944,972 | 7/1960  | Welsh -----             | 252—32.7    |
| 3,004,996 | 10/1961 | Arakelian -----         | 260—429.9   |
| 3,290,347 | 12/1966 | Miller -----            | 260—429.9   |
| 3,515,712 | 6/1970  | Goldsmith -----         | 260—429.9 X |

TOBIAS E. LEVOW, Primary Examiner

H. M. S. SNEED, Assistant Examiner

U.S. Cl. X.R.

252—32.7; 260—429 K, 435, 439 R, 953